

## UNITED STATES PATENT OFFICE.

VERN C. BARTLETT, OF JOPLIN, MISSOURI.

BATH OR FLUX FOR PREVENTING CORROSION OR RUSTING OF MOTOR-VEHICLE  
WHEEL RIMS AND WIRE WHEELS.

No Drawing.

Application filed September 12, 1922. Serial No. 587,810.

*To all whom it may concern:*

Be it known that I, VERN C. BARTLETT, a citizen of the United States, residing at Joplin, in the county of Jasper and State of Missouri, have invented new and useful Improvements in Baths or Flux for Preventing Corrosion or Rusting of Motor-Vehicle Wheel Rims and Wire Wheels, of which the following is a specification.

10 The object of my said invention is the provision of an economical and efficient bath or flux for treating wheel rims that carry rubber tires, whereby the formation of rust on said rims is effectively prevented.

15 To the attainment of the foregoing, the invention consists in the improvement as hereinafter described and definitely claimed.

In the best practice of my invention of which I am cognizant I first boil the rim, 20 demountable rim, or the wire wheel in a strong solution of caustic soda, this to eliminate paint, rust and the like therefrom. I then scrub the rim or wheel, and rinse the same to remove all alkali. The rim or the 25 wheel is then immersed in commercial muriatic acid with a view to effectively removing therefrom all foreign substance. The rim or the wheel is then placed in a bath or flux composed of the following ingredients 30 combined in substantially the proportions stated, viz:

|                   | Per cent. |
|-------------------|-----------|
| Zinc chloride     | 48        |
| Glycerine         | 4         |
| 35 Zinc sulfate   | 2         |
| Water (distilled) | 46        |

The rim or the wheel is let remain in the bath or flux defined for an appropriate 40 period of time, after which the rim or the wheel is removed from the bath and is

quickly thereafter immersed in pure molten tin (preferably block tin). In this way the rim or the wheel will be uniformly and smoothly coated with tin which in virtue of being fluxed on by the bath defined will strongly adhere to and will not scale or flake off with the result that the rim or the wheel will be permanently and adequately protected against rust or corrosion.

In the case of wire wheels, the described coating of tin also serves to permanently set the spokes so that loosening of the spokes will be precluded. I would also have it understood that when deemed expedient copper filings may be mixed with the pure tin for the coating of wire wheels in order to impart an attractive golden or bronze color to the wheels.

My improvement as hereinbefore set forth is not to be confounded with the use of zinc on automobile and aeroplane wheel rims, zinc because of its hardness being liable to oxidize and flake off whereas tin because of its soft quality will give to vibration and shock and bends and will adhere to the metallic parts that it covers and protects.

Having described my invention, what I claim and desire to secure by Letters Patent, is:—

1. A solution for the purpose described consisting essentially of zinc chloride, glycerine, zinc sulfate, and water.

2. A solution for the purpose described 75 consisting essentially of zinc chloride, glycerine, zinc sulfate, and water; zinc chloride 48 per cent, glycerine, 4 per cent, zinc sulfate, 2 per cent, and water 46 per cent.

In testimony whereof, I affix my signature.

VERN C. BARTLETT.